

## UNITED STATES PATENT OFFICE

2,517,852

AIRPLANE FABRIC AND METHOD OF  
MANUFACTURING AIR FRAMES

Alfred Dreyling, South River, N. J., and Charles William Johnson, Flint, Mich., assignors to E. I. du Pont de Nemours & Company, Wilmington, Del., a corporation of Delaware

No Drawing. Continuation of application Serial No. 436,412, March 27, 1942. This application December 5, 1946, Serial No. 714,128.

5 Claims. (Cl. 244—123)

1

This invention relates to an improved coated airplane fabric and more particularly to a system or process of preparing airplane parts using such coated airplane fabric which greatly shortens this time-consuming step in the manufacture of aircraft.

This application is a continuation of copending application Serial No. 436,412, filed March 27, 1942, now abandoned.

In the construction of modern aircraft, both for civil and for military purposes, even for ships which are substantially all metal, numerous parts, for example, control surfaces such as rudders, elevators, flaps and ailerons, are provided with a fabric surface. In the specification and claims, such parts are called "air frames" for simplicity. In practice an uncoated fabric is tightly stretched over the air frame by tailoring onto the frame a fabric "sock" which is deliberately prepared under-size in order to make it more tightly fitting. A clear cellulose derivative "dope," usually two brush coats, is then applied to the fabric surface to lay the nap of the fabric and to function as a size coat for subsequently applied top coats. Two to four clear cellulose derivative coatings are then sprayed over the base coat followed by two to four cellulose derivative coatings containing coloring matter. Each coat is dried and sometimes sanded before the application of the following coat. This system, which requires a considerable number of operations, presents many application problems and, in addition, is undesirably time-consuming particularly in the present-day "production line" construction of military aircraft where a single "bottle neck" serves to greatly retard maximum production.

It has been proposed to predope the fabric prior to tailoring it onto the air frame and tests have been carried out in which the fabric has been precoated with conventional "dope" coating compositions. However, this method provides a coated fabric which is quite boardy and which is difficult to handle and tailor to the air frame, thereby counteracting any advantage that might accrue through the precoating of the fabric prior to its use in the aircraft factory.

The process of the present invention, however, overcomes these disadvantages and provides a method for greatly speeding up the production of military aircraft.

This invention, therefore, has as a primary object the provision of a method for covering air frames and predoping airplane fabric which affords material saving in time in the aircraft factory, thereby greatly increasing the production rate of aircraft manufacture by reducing the doping schedules.

2

A further object is the reduction in the number of coatings and other operations required in finishing fabric surfaces which are essential in the manufacture of military and civil aircraft.

5 Another object is the provision of a method for coating airplane fabric which provides satisfactory tautening of the fabric after it is attached to the air frames.

Another object is the provision of a composition which affords a smoother finish by more effectively laying the nap and which also avoids the necessity for sanding.

Another object is the provision of a system for finishing airplane fabric which provides greater suppleness and pliability of the fabric, thereby greatly assisting in tailoring the fabric to the air frames.

A still further object is the provision of a composition which provides a "discontinuous" film adjacent to the fabric which subsequently is rendered continuous by the application of top coat dope coatings containing solvents for the "discontinuous" film.

A still further object of the invention is the provision of a pliable predoped airplane fabric which greatly facilitates the tailoring of the fabric to the air frames and which affords better working properties.

These objects are accomplished by the application of a cellulose derivative emulsion preferably free of resin and wax to the surface of an airplane fabric, said emulsion being so formulated as to be totally deposited as a precipitated film which is discontinuous in nature.

The following examples are given by way of illustration only and no limitations are intended thereby except as indicated in the appended claims.

## 40 Example 1.—Cellulose nitrate emulsion (spray coating)

|    |                                 | Per cent<br>by weight |
|----|---------------------------------|-----------------------|
| 45 | First portion:                  |                       |
|    | Cellulose nitrate <sup>1</sup>  | 29.0                  |
|    | Water                           | 10.6                  |
|    | Butyl alcohol                   | 5.8                   |
|    | Butyl acetate                   | 23.4                  |
|    | Methyl ethyl ketone             | 11.5                  |
|    | Castor oil                      | 5.8                   |
| 50 | Second portion:                 |                       |
|    | Polyvinyl alcohol               | 0.6                   |
|    | Water                           | 12.7                  |
|    | Isopropyl naphthalene sulfate   | 0.2                   |
|    | High solvency petroleum naphtha | 0.4                   |
|    |                                 | 100.0                 |

<sup>1</sup> The viscosity characteristic of the nitrocellulose is 5 seconds determined in accordance with A. S. T. M. Specification D-301-33, Formula A.

The first portion was prepared by charging the ingredients into a kneading machine such as a Werner and Pfleiderer mixer, in the proportions indicated and kneading for approximately 1½ hours or until the mass becomes smooth and free from undissolved material, after which the charge was removed from the mixer. The second portion is conveniently prepared by means of a rapid agitator mixer, whereby a homogeneous dispersion is secured. The second portion was then charged into a kneading machine and the first portion added gradually during continued kneading. This kneading action was continued until emulsification was complete; i. e., when the first portion was dispersed as globules within the second portion which forms the continuous phase. By complete emulsification is meant when a uniform predetermined particle size is reached which may be determined by microscopic examination. In the present instance the particle size was approximately 12 microns.

The emulsion composition was thinned with water in the ratio of 3 parts of emulsion to 1 part of water and two coats of the thinned material applied by spraying onto airplane fabric consisting of Grade A Flightex mercerized cotton sheeting having a thread count of between 80 and 84 in both the warp and filler direction and weighing approximately 4.0 oz. per square yard. The first coat was dried at room temperature for about 45 minutes before application of the second coating. The resulting finish was a white-appearing, discontinuous coating which leaves the cloth very pliable and supple and readily adapted to tailoring onto an air frame. The weight of the coating when dried was approximately 1 oz. per square yard.

The fabric coated as described above was stretched over a frame and one double coat of the following conventional pigmented dope thinned as described was applied by spraying.

|                                                | Percent by weight |
|------------------------------------------------|-------------------|
| Castor oil                                     | 0.5               |
| Nitrocellulose <sup>1</sup>                    | 7.6               |
| Dibutyl phthalate                              | 3.6               |
| Lead chromate pigment                          | 5.0               |
| Ethyl alcohol                                  | 4.0               |
| Methyl ethyl ketone                            | 7.3               |
| Ethyl acetate                                  | 7.7               |
| Butyl acetate                                  | 18.6              |
| Butyl alcohol                                  | 4.0               |
| High solvency petroleum naphtha (135°-190° C.) | 5.8               |
| High solvency petroleum naphtha (95°-135° C.)  | 35.9              |
|                                                | 100.0             |

<sup>1</sup> The viscosity characteristic of the nitrocellulose is 10 seconds determined in accordance with A. S. T. M. Specification D-301-33, Formula A.

Before spraying this composition onto the pre-coated fabric, it was thinned with equal parts of the following thinner:

|                                                | Percent by weight |
|------------------------------------------------|-------------------|
| Butyl acetate                                  | 20.5              |
| Methyl ethyl ketone                            | 8.6               |
| Ethyl alcohol (denatured)                      | 9.5               |
| Butyl alcohol                                  | 9.0               |
| High solvency petroleum naphtha (135°-190° C.) | 2.3               |
| High solvency petroleum naphtha (95°-135° C.)  | 27.6              |
| Petroleum naphtha (88°-131° C.)                | 22.5              |
|                                                | 100.0             |

This treatment caused the base coat to become a continuous film by action of the solvents present in the top coat which dissolved and coalesced the discrete particles comprising the base coat. 5 Considerable shrinkage occurred upon evaporation of the volatile solvents, thus affording the desired tautening effects.

10 A tautness determination by McGowan Tautness Meter showed a deflection of .091 inch which represents a satisfactory tautness.

The McGowan Tautness Meter is described in "Physical and Chemical Examination of Paints, Varnishes, Lacquers and Colors," page 430 by H. A. Gardner, 9th ed., 1939.

15 The precoated fabric of the present invention when coated with one or more conventional dope compositions such as illustrated above will provide a tautness such that a deflection of less than .110 inch is obtained on the McGowan Meter, which is satisfactory for the purpose described.

*Example 2.—Cellulose nitrate emulsion (for knife coating)*

|                                | Per cent by weight |
|--------------------------------|--------------------|
| First portion:                 |                    |
| Cellulose nitrate <sup>1</sup> | 25.0               |
| Water                          | 12.3               |
| Methyl ethyl ketone            | 35.0               |
| Toluol                         | 6.0                |
| Tricresyl phosphate            | 5.0                |
| Second portion:                |                    |
| Polyvinyl alcohol              | 0.6                |
| Isopropyl naphthalene sulfate  | 0.2                |
| Water                          | 15.9               |
|                                | 100.0              |

<sup>1</sup> The viscosity characteristic of the cellulose nitrate is 5 seconds determined in accordance with A. S. T. M. Specification D-301-33, Formula A.

40 This composition was prepared by the procedure shown for the preparation of the emulsion of Example 1.

45 100 parts by weight of the above composition were thinned with 12 parts by weight of water and the thinned material then continuously knife-coated by conventional methods onto a water-dampened airplane fabric traveling at the rate of 7.5 yards per minute. The coating was dried by passing the coated fabric through a drying tunnel at the temperature of 180° F. Two coats were applied in this manner. The resulting coating which was discontinuous gave a product which was soft and pliable and easily tailored onto an air frame. The coated fabric was stretched tightly over a frame and one spray coat of the conventional pigmented dope shown in Example 1 applied by spraying. This treatment gave a final finish which was uniformly smooth and caused a satisfactory tautening of the fabric on the frame.

50 In addition to the cellulose nitrate shown in the examples, other water insoluble film forming cellulose derivatives such as ethyl cellulose, cellulose acetate and the mixed esters, for example, cellulose acetobutyrate and cellulose acetopropionate may likewise be employed with proper plasticizers and suitable volatile solvents so proportioned with regard to the water in the emulsion composition as to provide a discontinuous finish upon evaporation of the volatile constituents. Cellulose acetate and ethyl cellulose are not preferred for airplane fabric coatings because of their tendency to lose tautness but they are operable in the process and may be useful for coat-

ing other types of fabrics. In any event, it is necessary and critical to the success of the invention that the film be precipitated to afford the desirable discontinuity in the undercoat. The solids composition of the coating are preferably similar to conventional dope compositions. The plasticizer ratio should be relatively low, preferably in the proportion of 10 parts of nitrocellulose to 1 to 4 parts of plasticizer. Any substantially higher proportion of plasticizer causes undesirable reduction in tautening effects when the top coats are applied and dried.

The emulsion composition as employed in the improved system of the present invention for finishing fabric parts of aircraft should be substantially free of resin and wax since materials of this type tend to cause embrittlement of the finish, a tendency which cannot be tolerated for the present purpose where a high degree of flexibility and pliability are of paramount importance.

It is also necessary to include in the emulsion composition sufficient of non-solvent for the cellulose derivative, preferably water, to cause precipitation of the nitrocellulose whereby a film of discontinuous nature is secured. To accomplish this, the non-solvent portion of the volatile vehicle should be present in an amount at least equal to the active solvent portion. Preferably the non-solvent content will be about 1½ to 3 times that of the solvent portion depending largely upon the solvent power and evaporation rate of the solvent portion of the vehicle.

The active cellulose derivative solvents employed in the compositions of the invention should not be completely miscible or soluble in water and in general it is preferred that they be not more than about 30% miscible with water. Furthermore, the evaporation rate of these solvents should be at least equal to and preferably greater than that of water or other non-solvent comprising that part of the vehicle in order that the cellulose derivative may be substantially completely precipitated during evaporation of the volatile vehicle and not become the more residual part of the volatile vehicle to cause coalescence of the cellulose derivative, thereby forming a continuous film. If the volatile vehicle is prepared in accordance with the above limitations, the resulting film when applied to a fabric base will be discontinuous as hereinafter defined. For compositions in which the cellulose derivative is cellulose nitrate, ethyl acetate, methyl ethyl ketone, butyl acetate and methyl isobutyl ketone are satisfactory.

The compositions adapted for the purposes of the present invention may, as illustrated in the examples, contain aliphatic and aromatic hydrocarbon diluents such as toluene, benzol and petroleum naphthas such as gasoline fractions. Alcohols, preferably those which are not completely miscible with water, may also be included in the volatile vehicle.

In some instances where a higher degree of water-resistance is desired, it is possible to include in the emulsion composition which may contain water soluble emulsifying agents, such as polyvinyl alcohol, a small proportion of an insolubilizing agent such as stearato chromic chloride described in U. S. Patent 2,273,040 to Ralph K. Iler or dimethylol uron dimethyl ether as described in co-pending application S. N. 438,949, now Patent No. 2,373,135 to Maxwell. In preparing the emulsion, such as Example 1, which

may be modified by the inclusion of the uron derivative, it has been found necessary in order to obtain satisfactory stability of the emulsion to incorporate the insolubilizing agent in the first portion and the aluminum chloride or other catalyst in the second portion of the emulsion.

It is also possible, and in some cases preferable, to apply the emulsion coating directly to a previously wetted fabric since this expedient may facilitate deposition by precipitation of the discontinuous type film.

While in some cases satisfactory results can be obtained by the use of a single top coat, it is usually preferable to apply two or more dope coats to afford better durability and to increase tautness.

Although not required for the successful operation of the invention, the fabric carrying the precipitated coating may be passed through heated polished rolls under pressure to smooth out the coating thereby contributing to the smoothness of the final finish.

The primary advantage of the invention is the marked saving in time and labor required at the airplane factory for finishing parts which involve the use of fabric covering. This is particularly important in the manufacture of military aircraft where all bottle necks tending to retard production must be obviated. The new process permits desirable reduction in the number of operations in the preparation of the coated fabric. The practice of the present invention permits the elimination of at least one dope coat in the finishing schedule and in some instances satisfactory results are obtained with the elimination of as many as 3 to 4 dope coats from the schedule. The new system affords satisfactory tautness in the finished fabric and durability in service is also at least equal in all respects to that secured by older methods. The new method of predoping the fabric more completely lays the nap, thus avoiding necessity of sanding operations, and provides a finish which is smoother than that obtained by other predoping methods. The fabric coated in accordance with the present invention carries a discontinuous film which affords superior pliability and suppleness, thereby facilitating tailoring of the fabric to the air frames. This also contributes greatly to the speeding up of operations and ultimate increase in aircraft production.

In the description and appended claims, a "discontinuous" coating is meant to define a coating which results from the precipitation of the cellulose derivative by the presence of an excess amount of non-solvent for the cellulose derivative during evaporation of the solvent vehicle, the resulting film after drying consisting substantially of noncoalesced, discrete particles or disconnected aggregates of small particles.

It is apparent that many widely different embodiments of this invention may be made without departing from the spirit and scope thereof; and, therefore, it is not intended to be limited except as indicated in the appended claims.

We claim:

1. The process of manufacturing airplane air frames which comprises coating a strong light-weight woven fabric with an aqueous emulsion of a cellulose derivative, the oil phase of which contains the cellulose derivative and a solvent, the evaporation rate of the solvent being greater than that of the water allowing the volatile vehicle to evaporate leaving a discontinuous coat-

ing of discrete particles on the fabric, the said vehicle containing from about 1 to 4 parts of a solvent plasticizer for each 10 parts of the cellulose derivative, tailoring the coated fabric into a sock, fitting the same tightly over the air frame, and subsequently shrinking the said fabric to a tautness deflection of less than about .110 inches by treating the said cellulose derivative with a solvent therefor.

2. The process of claim 1 in which the cellulose derivative is cellulose nitrate.

3. The process of claim 1 in which the water is present in amount at least equal to the amount of solvent.

4. The process of claim 1 in which the non-solvent is present in amount equal to about 1½ to 3 times that of the solvent.

5. A predoped airplane fabric characterized by a high degree of suppleness and pliability having a precipitated coating thereon of a composition having the following formula:

|   |                               | Parts by weight |
|---|-------------------------------|-----------------|
|   | Cellulose nitrate             | 29.0            |
|   | Castor oil                    | 5.8             |
|   | Polyvinyl alcohol             | 0.6             |
| 5 | Isopropyl naphthalene sulfate | 0.2             |

ALFRED DREYLING.

CHARLES WILLIAM JOHNSON.

REFERENCES CITED

The following references are of record in the file of this patent:

UNITED STATES PATENTS

| Number    | Name         | Date          |
|-----------|--------------|---------------|
| 1,357,541 | Cahill       | Nov. 2, 1920  |
| 1,394,890 | Gault        | Oct. 25, 1921 |
| 1,552,808 | Sulzer       | Sept. 8, 1925 |
| 1,940,212 | Given et al. | Dec. 19, 1933 |
| 2,336,266 | Lester       | Dec. 7, 1943  |
| 2,356,927 | Grossman     | Aug. 29, 1944 |